

Patented May 22, 1928.

1,670,463

# UNITED STATES PATENT OFFICE.

JOHN WESLEY MARDEN, OF EAST ORANGE, NEW JERSEY, ASSIGNOR TO WESTINGHOUSE LAMP COMPANY, A CORPORATION OF PENNSYLVANIA.

## ELECTRON-EMISSION MATERIAL AND METHOD OF PREPARATION.

No Drawing.

Application filed April 11, 1923. Serial No. 631,366.

This application is a continuation-in-part of my copending application Serial No. 504,154, filed Sept. 29, 1921, production of rare metals and alloys thereof and assigned 5 to the Westinghouse Lamp Company.

This invention relates to electron-emission material and the preparation thereof and more particularly to the employment of alloys of aluminum and metals such as thorium, uranium, zirconium and the like for activating such material and for other purposes.

An object of my invention is the preparation of activated filamentary material by incorporating efficient metallic electron-emission material into refractory metal, said electron-emission material being first combined with another metal as a carrier and protector of the electron-emission material.

Another object of my invention is the employment of alloys of aluminum with refractory rare metals for activating material for electron-emission purposes and the like.

A further object of my invention is the activation of metals of the tungsten class including tungsten, molybdenum, platinum, tantalum and the like by incorporating therewith an alloy of aluminum and an electron-emission material such as thorium, uranium, titanium, zirconium or the like and subsequently eliminating the aluminum therefrom by vaporization.

A still further object of my invention is the preparation of alloys of aluminum and refractory rare metals such as thorium, uranium, zirconium, titanium and the like for application to an element of an electron device, whereby activation of an electron-emitting filament therein may be accomplished 40 by the rare metal, simultaneously with a clean-up action by the aluminum.

Other objects and advantages of the invention will become apparent as the description proceeds.

In the copending application of Marden and Rentschler Serial No. 583,377, filed August 21, 1922, rare metal alloys and method of preparation and assigned to the Westinghouse Lamp Company, is disclosed a method 50 of preparing activated molybdenum by incorporating a small proportion of metallic thorium therein prior to pressing, sintering and working the same to the desired form. The method disclosed has given good results, 55 but it entails the use of metallic thorium

which is not only difficult and expensive to prepare, but readily oxidizes and is easily contaminated by moisture, nitrogen and other materials.

In the copending application of C. T. Ulrey, Serial No. 577,021, filed July 24, 1922, manufacture of electron-emitting devices and the like and assigned to the Westinghouse Lamp Company, is disclosed a method of activating a cathode, adapted for electron-emission purposes, by heating an anode disposed adjacent thereto and composed, at least partly, of thorium so that some of said thorium is distilled or sputtered from said anode to the cathode for increasing its electron-emissivity. This method of activation is satisfactory, but likewise entails the use of metallic thorium which, as before noted, is expensive, difficult to prepare and readily contaminated by other substances.

According to my invention, I accomplish the results obtained according to the aforementioned applications, but instead of using metallic thorium, I propose to use an alloy, solid-solution, mixture or compound of thorium or other material with high electron-emitting properties, such as uranium, zirconium or the like, with aluminum, which serves as a protector, of the thorium or other rare metal, from contamination and holds it in a form in which it may be conveniently utilized for the purposes desired. The alloy of the electron-emitting metal and aluminum may be prepared in a manner similar to that disclosed in my copending application before referred to, Serial No. 504,154, filed September 29, 1921, production of rare metals and alloys thereof and assigned to the Westinghouse Lamp Company.

After preparing the desired aluminum alloy, according to said application, the same may be powdered and mixed in the desired proportion with the selected refractory metal to be activated, for example, molybdenum. The mixture may then be pressed into the form of a cake or slug, preferably square in cross section. It may then be sintered in a vacuum or heat-treated to cause the particles to coalesce to form a homogeneous slug adapted to be worked to the desired size and shape. The sintering is preferably continued at a high enough temperature, slowly enough and for a sufficient length of time to free the alloy from the aluminum by vaporization.

Instead of producing activated material in such manner, an electron-emitting cathode may be activated in place in a radio tube or the like, by applying to an adjacent plate or anode in said tube, a coating of powdered thorium aluminide or other alloy or mixture of aluminum with a metal having good electron-emissivity.

Said material may be applied by mixing 10 the same with a suitable binder, such as an amyl-acetate solution of nitrocellulose, and painting the mixture upon the anode or, if desired, directly on the cathode. Instead of applying the alloy by painting, the same 15 may be formed of a strip or clip and fastened to said plate or anode in any suitable manner, as by pasting, crimping or welding. The adjacent filament or cathode may then be activated by sputtering, vaporization or 20 transfer of the electron-emission material from the plate to the filament, by heating in any desired manner, for example, by electron-bombardment such as described in the aforementioned copending application of 25 C. T. Ulrey.

The following detailed description is a disclosure of the use of thorium-aluminum alloys for producing activated molybdenum, but alloys of aluminum and other electron-emission material for example, uranium and zirconium, may be prepared and used for similar purposes. The same or a similar process may be employed for preparing activated tungsten, or other metal of the 30 tungsten class.

The thorium-aluminum alloy may be prepared according to my aforementioned application Serial No. 504,154, of which this application is a continuation-in-part or, 40 briefly, as follows.

A halide salt of thorium, for example, thorium-ammonium-chloride is prepared, preferably by the process disclosed in my copending application Serial No. 498,397, 45 filed September 3, 1921, preparation of metals and their halides and assigned to the Westinghouse Lamp Company. That process involves the treatment of the hydrated salts of the rare metals with a displacing substance, for example, ammonium chloride 50 added to a solution thereof. The solution may then be evaporated to dryness to eliminate the water and part of the ammonium chloride.

The residue, which is thorium-ammonium-chloride, may be placed in a graphite crucible and covered with a previously fused and cooled mixture of sodium and potassium chloride or fluoride or other halogen alkali 60 compounds. The crucible, with the mixture therein, may be placed in a furnace and the temperature raised until the mixture is fused to a clear liquid.

In order to prevent oxidation, a slow current of carbon tetrachloride vapor or other

chlorine-containing reducing agent, may be passed into the top of the crucible. After complete fusion, approximately several times the weight of aluminum necessary to make the reduction is added to the fused 70 mixture, a small quantity at a time. The heating is continued for about 20 minutes or until the thorium-aluminum alloy collects and separates itself, from the fused salt or slag, as a button or slug at the bottom of the 75 crucible. This button after being broken away and crushed into a fairly fine powder, may be washed in water and purified in any desired manner to recover the thorium-aluminum alloy or aluminide. It is deemed 80 preferable to purify the powder by treating with a fairly strong solution of caustic soda to dissolve out the excess of aluminum not alloyed with the thorium.

The residue, which is thorium aluminide 85 ( $\text{Th}_3\text{Al}_4$ ), may then be washed with water and treated with dilute acid, for example, hydrochloric acid, to remove all the caustic soda and acid-soluble materials from the alloy. After filtering and drying, the aluminide may be used for activating purposes, as will be subsequently described, for hardening aluminum by forming aluminum alloys containing small proportions of refractory rare metals or for any desired purpose. 90

The powdered alloy or aluminide may be mixed in the desired proportion with powdered molybdenum or the like. In order to prepare activated material or material having high electron-emissivity, it is only 100 necessary to use a small proportion of the thorium alloy with a molybdenum, tungsten or other refractory metal powder which may be used. For example, from  $\frac{1}{2}$  to 1%, by weight, of the alloy is sufficient to give good activation. Such a mixture may then be pressed into a cake or slug, preferably square in cross section, and considerably longer than the cross sectional dimensions thereof. Slugs for experimental work 3 110 inches long and  $\frac{1}{16}$  inch square in cross section, may be used, but, in practice, it is preferable to use slugs about  $\frac{1}{4}$  inch to  $\frac{3}{4}$  inch square and 8 inches long.

The slug may be sintered to a high temperature in a high-frequency induction furnace, that is, for example, the pressed slug may be placed on a sheet of molybdenum or other refractory metal and inserted in a sintering furnace of the type described in the copending application of Marden and Rentschler Serial No. 488,229, filed July 28, 1921, a process of manufacturing metals and their uses, and assigned to the Westinghouse Lamp Company. 115

Such sintering is optional and is recommended for slugs of small size only, or where such have been formed too weak for the heat treatment, later described, without sintering. If the material has been sufficiently 120 125 130

sintered and the purity of the same maintained, by causing the sintering to be accomplished by a high vacuum, the current may then be shut off and the resultant product permitted to cool within the furnace while maintaining the high vacuum.

5 A pressed slug either sintered, or the optional sintering operation having been omitted, may then be heat-treated, at a temperature nearly high enough to melt it, in a specially-constructed furnace, for example, such as that described and claimed in the copending application of Rentschler and Marden Serial No. 488,230, filed July 28, 15 1921, furnaces and assigned to the Westinghouse Lamp Company. Any furnace wherein the slug may be heated in an inert environment, such as a high vacuum, to nearly the melting point thereof, may be employed.

20 The resulting alloy will be found to be strongly coherent, dense, tough and less liable to crack on unequal heating and cooling and to have lost entirely all of its brittleness, so that, when it is heated red-hot, it 25 may be readily swaged, rolled, hammered or drawn to render it ductile. The slug may be rolled to size or swaged hot until round in cross-section and then drawn down to the desired size of wire, in a manner well known 30 for working molybdenum, if such is used, or for working tungsten or other refractory metal, if such is used, instead of molybdenum.

The sintering or heat treatment previously 35 described may be conducted at such high temperature as to eliminate the aluminum content by distillation or vaporization thereof. The thorium aluminide, or other alloy used, will not dissociate until the slug has 40 been substantially entirely rid of gases, which prevents the thorium, after the aluminum has been vaporized therefrom, from gas contamination, whereby it is left in a metallic condition alloyed with the molybdenum, 45 tungsten or whatever refractory metal, the thorium-aluminum alloy has been added to. Wire formed from such an alloy, is an efficient electron-emission material, in fact as good as pure thorium, even though the thorium content may be very small. The aluminum 50 content has a purifying and scavenging action on the product, whereby an alloy is obtained which is more free from oxides and other deleterious impurities than those heretofore employed.

Activation by means of thorium aluminide or other thorium-aluminum alloy may be effected, in an electron tube or the like, by applying the same upon the plate or anode 55 therein, by mixing the same in a powdered form with a suitable vehicle or binder, such as an amyl-acetate solution of nitro-cellulose, and painting the mixture upon the plate. An alternative method may consist in applying the aluminide to the plate or

anode in the form of a clip or strip fastened thereto in any suitable manner. The plate may then be heated to a high temperature in any convenient manner, for example, as described in the aforementioned application 70 of C. T. Ulrey, whereby the thorium content is transferred or sputtered from the plate to the electron-emitting filament, to cause the same to become activated. The aluminum content, in this instance, may serve a 75 double function of preserving the thorium from contamination until it is desired to use the same for activating purposes and also act as a clean-up agent or vacuum-improving substance, when the same is heated, and thereby obviate the necessity of using additional aluminum or some other clean-up material, such as magnesium, calcium or the like, for that purpose.

Although the thorium aluminide or thorium-aluminum alloy has been heretofore described as a means for activating filamentary material or the like, alloys of aluminum and refractory rare metals, such as zirconium, titanium, uranium, molybdenum, tungsten, 90 thorium and the like, may be employed for other purposes wherein the refractory rare metal is used merely as a hardener and strengthener in the aluminum, to give the same desirable properties for castings which 95 could be used in automobiles, aeroplanes and other devices needing light metals of high tensile strength and where the parts could be cast.

The desired alloy may be prepared as heretofore described, although preferably more aluminum is used so that the proportion of the rare metal, for example, zirconium, is relatively small. Aluminum holds about 8% of zirconium, after which crystals, having 100 about 30% aluminum in them and corresponding to the formula  $Zr_3Al_4$  separate from the mass. An 8% zirconium-aluminum alloy has a Brinell hardness of about 54, a Shore hardness of about 12, an elastic limit of 13,500 pounds per square inch and a tensile strength of about 27,000 pounds per square inch. This is about the same tensile strength and hardness as a copper-aluminum alloy, having perhaps about 10 to 12% copper. 105 A 4% zirconium-aluminum mixture or alloy has a hardness and tensile strength corresponding to about a 6% copper-aluminum alloy.

Although I have described what I now 120 consider to be the preferred methods of practicing my invention, in connection with certain specific alloys or mixtures, it is to be noted that the alloys mentioned are merely illustrative and that my invention is adapted 125 for alloys of aluminum with the refractory rare metals for electron-emission purposes or general use.

What is claimed is:

1. The process of activating refractory 130

metal for electron-emission purposes comprising incorporating a small proportion of a powdered aluminum alloy of electron-emission metal with powdered refractory metal, pressing the mixture into a slug, heat-treating the same and working to the desired form.

2. The process of preparing a thorium-molybdenum alloy comprising heat-treating a pressed mass of a mixture of molybdenum powder and thorium-aluminide powder in a desired proportion to cause the particles thereof to be firmly welded together, said heat-treating operation being conducted in

15

a vacuum.

3. The process of alloying or forming a coherent ductile alloy of thorium and molybdenum comprising mixing powdered thorium-aluminide and powdered molybdenum in the desired proportion, pressing the same in the form of a slug and heat-treating until the aluminum is eliminated therefrom and the particles of thorium and molybdenum become firmly welded together.

20 4. The method of making alloys or mixtures comprising mixing an alloy of thorium and aluminum in powdered form with pow-

dered molybdenum, pressing the mixture into the form of a slug and heat-treating to vaporize the aluminum therefrom and cause 30 the particles of the remaining alloy to weld firmly together, said heat-treating operation being conducted in an inert environment.

5. The method of producing refractory alloys for electron emission purposes which 35 comprises activating a filament by the addition of an alloy of aluminum and a metallic electron emission material and purifying by heating the filament in a vacuum to eliminate the aluminum therefrom.

6. The method of activating refractory metal filaments consisting in adding thereto an alloy of thorium and a vaporizable metal and heating the filament to eliminate the vaporizable metal.

7. The method of activating refractory metal filaments comprising associating therewith, an alloy of thorium and aluminum and heating the filament to eliminate the aluminum therefrom.

In testimony whereof, I have hereunto subscribed my name this 10th day of April 1923.

JOHN WESLEY MARDEN.